

# UNITED STATES PATENT OFFICE.

HARRY L. HAAS, OF NEW YORK, N. Y., ASSIGNOR OF ONE-FOURTH OF HIS  
RIGHT TO ALEXANDER LEVETT, OF SAME PLACE.

## SOLUTION FOR NICKEL-PLATING.

SPECIFICATION forming part of Letters Patent No. 230,872, dated August 10, 1880.

Application filed February 18, 1880.

*To all whom it may concern:*

Be it known that I, H. L. HAAS, of the city, county, and State of New York, chemist, have invented certain new and useful Improvements 5 in the Art of Nickel-Plating, consisting of a new process of securing the electro-deposition of nickel.

In order to enable others to practice my invention, I do hereby declare that the following 10 is a full and exact description thereof.

My invention relates to an improvement in the art of nickel-plating; and it consists in the employment of a solution containing formate of nickel, with excess of acid, as herein- 15 after more fully set forth.

I use as an anode an ordinary cast nickel plate prepared in any of the usual methods. I take the green oxide of nickel, well known as an article of commerce, or I form oxide of 20 nickel by dissolving commercial nickel (the purer the better) in nitric acid, thereby forming a nitrate of nickel. This should be evaporated to dryness, and when heated leaves the green oxide of nickel. The oxide of nickel is 25 then dissolved in formic acid. The resulting solution is the formate of nickel. This solution should be diluted. I have obtained excellent results when such solution has a specific 30 gravity of 1.050, water being 1.000; but useful results may be accomplished within a wide range of strength of the solution, and good results may be obtained when the solution is much weaker than is above stated. The weaker the solution, however, the longer 35 time is required to obtain the deposit under the same conditions.

Formate of nickel is capable of crystallization, and therefore can be manufactured and sold in a cheap and convenient form ready for 40 use, and could be used by any nickel-plater simply by dissolving it in water.

When the solution is prepared the anode and cathode are immersed in it, and the electric battery is applied. With the solution of 45 the specific gravity of 1.050 I have used a Daniell battery of three cells or a Bunsen battery of one cell.

The action of the battery upon the formic acid in the solution of the formate of nickel is 50 such that carbonic-acid gas and oxygen go to

the anode and metallic nickel and hydrogen go to the cathode, and the nickel is deposited.

Instead of using the oxide of nickel in forming the solution, the hydrated oxide of nickel may be employed, and such hydrate may be 55 precipitated from any solution of nickel by an alkali, such as potash. The hydrate so formed may be washed, and when dried is dissolved in the formic acid.

It is not necessary that the solution which 60 I employ should be free from potash, soda, lime, or alumina, or even from traces of nitric acid, for articles which have been cleaned by such alkalies or acid, and which are left by careless workmen with a little of such sub- 65 stances adhering, will not affect my solution.

The result of using the solution aforesaid is the electro-deposition of a firm, coherent, and continuous deposit of clean and white nickel, 70 and the use of such solution possesses the following advantages over any previous process with which I am acquainted:

First, it is an acid solution, and the battery-current does not affect it within any reasonable limits of intensity. 75

Second, it contains no ammonia. Hence there is no liability to decomposition and the liberation of free ammonia by the use of a high battery power, which impairs the value 80 of other solutions.

Third, the process is a continuous one, and the solution needs no replenishing with salts of nickel, the nickel being supplied from the anode. 85

Fourth, no precautions need be taken to see that the solution is free from the presence of potash, soda, alumina, lime, or nitric or other acid.

Fifth, the deposit may be of any thickness, 90 and will always be firm, flexible, and white.

It will be perceived that the basis of my invention is the use of a diluted solution of formate of nickel containing an excess of acid, and that this solution requires less care and is 95 cheaper in management than any solution with which I am acquainted.

When the formate of nickel is used as above specifically described the only precaution which it is necessary to observe is that the ar- 100

ticles to be plated should be very clean, and especially free from grease.

The deposit may be made by my solution upon brass, copper, iron, or tin, and, so far as I know, upon any metal.

I am aware that in nickel-plating an alkaline solution containing formate of nickel and ammonia has heretofore been employed, and I therefore lay no claim to such invention.

10 My solution contains formate of nickel with excess of acid, and no ammonia or double salts, and is therefore very different from the solution disclaimed.

What I claim, and desire to secure by Letters Patent, is—

In the art of nickel-plating, a solution containing formate of nickel with excess of acid, and diluted to the required strength, substantially as described, and for the purpose set forth.

HARRY L. HAAS.

Witnesses:

SAML. R. BETTS,  
J. L. HAAS.